# EUROPEAN PATENT SPECIFICATION

(11) **EP 0 767 236 B1**
(45) Date of publication and mention of the grant of the patent: **27.06.2001**
(21) Application number: 96300983.2
(22) Date of filing: 13.02.1996
(51) Int. Cl.: C10M 169/04

(54) **Friction modification of synthetic gear oils**
Modifizierung der Reibung synthetischer Getriebeöle
Modification de la friction d'huiles synthétiques pour engrenages

(30) Priority: 04.10.1995 GB 9520295
(43) Date of publication of application: 09.04.1997
(73) Proprietor: ETHYL PETROLEUM ADDITIVES LIMITED, Bracknell, Berkshire RG12 2UW (GB)
(72) Inventor: Poat, Julia C., Bracknell, Berkshire, RG12 9PS (GB); Walters, David K., Camberley, Surrey, GU17 7TR (GB); MacPherson, Ian, Richmond, Virginia 23233 (US)
(74) Representative: Cresswell, Thomas Anthony

(56) References cited:
- EP-A- 0 501 527
- EP-A- 0 531 585
- EP-A- 0 578 435
- EP-A- 0 620 268
- WO-A-87/05927
- US-A- 5 089 156
- US-A- 5 250 122

## Description

This invention relates to improving the frictional characteristics of gear oils in which the base oil is, or contains a substantial quantity of, a synthetic poly-alpha-olefin oil (PAO).

PAOs possess good thermal stability and viscometric properties. However attempts to formulate PAO-based gear oils especially transmission oils for use in large vehicles equipped with manual transmissions of the synchroniser type pose special problems. Even though such lubricants contain additives for wear protection, corrosion protection, and other property improvements, the lubricants afford unsuitably low frictional properties in synchroniser-based transmissions and thus cause poor synchronisation of the gear changes. This negative aspect of such synthetic based gear oils is readily observed as low friction and noisy gear change in the Zahnradfabrik Friedrichshafen A.G. synchroniser test (described and referred to hereinafter as the "ZF Synchroniser test").

It has now been found possible to overcome this problem by means of small amounts of an additive which does not materially affect the other performance capabilities of the finished lubricant.

The additives used pursuant to this invention are overbased alkaline earth metal salts of oil-soluble sulfurised phenols or oil-soluble salicyclic acids. The metals of such salts preferably are those which have low toxicity and which present little or no concern from the environmental standpoint, namely, magnesium and calcium. However, the overbased barium and strontium salts can be used, if desired.

In accordance with one embodiment of this invention, there is provided a lubricant suitable for use as a gear oil lubricant for a manual transmission of the synchroniser type having a kinematic viscosity at 100° C in the range of 4 to 32 mm².s⁻¹ (cSt), and comprising:
a) a base oil comprising more than 40% by volume of hydrogenated poly-α-olefin oil; and
b) a friction improving amount in the range of 0.01 to 2wt% based on the total weight of the lubricant of at least one overbased alkaline earth metal sulphurised phenate or salicylate;
the lubricant being essentially free of any metal additive component other than the phenate or salicylate (i.e., the lubricant contains at most 100 ppm and preferably no more than 50 ppm of metal as one or more additive components other than said phenate or salicylate), and having on a weight basis a boron content, if any, of not more than 1,000 ppm, preferably not more than 300 ppm, and most preferably not more than 25 ppm. Typically, the lubricant does not contain any metal-containing component other than the phenate or salicylate, and has on a weight basis a boron content of not more than 300 ppm.

In one embodiment the lubricant has no boron additive content. In preferred embodiments the lubricant contains no metal additive component other than said phenate or salicylate.

Preferably the base oil (a) of the above gear lubricant comprises (i) at least 40%, and more preferably at least 50%, by weight of hydrogenated poly-alpha-olefin oil; (ii) 5 to 25% by weight of synthetic ester oil, and (iii) 0 to 55%, and more preferably 0 to 50% by weight of mineral oil. It will be seen that the mineral oil is an optional component of the base oil.

The present invention also provides the use, in a manual transmission of the synchroniser type, of the lubricant of the invention, to improve transmission performance during operation under service conditions. The lubricants can also be used to lubricate the axle or differential gearing system of the vehicle.

In the ZF Synchroniser test the beneficial increase in friction exhibited by finished gear lubricants of this invention manifests itself in a substantial increase in the number of cycles during which the test can be performed without poor synchronisation of the gear changes and/or with the coefficient of friction being greater than 0.065.

Preferably, the lubricant of the invention comprises a gear oil additive package such that the lubricant satisfies or exceeds the specifications for API GL-4 service. In satisfying or exceeding the specification for API GL-4 service, the finished lubricant satisfies the requirements for other performance specifications such as API GL-5, and including specifications not yet in being (or even envisioned) such as MT-1, PG2, API GL-7, and MIL-L-2105E or specifications of other countries such as comparable JIS gear oil standards, or the like. In other words the specifications of API GL-4 are to be considered minimum performance levels which the gear oil additive package (b) imparts to the finished lubricant. For example, if the requirements of the API GL-7 specification are more stringent than API GL-4, an additive package that provides a lubricant which satisfies the API GL-7 requirements inherently satisfies the minimum performance requirements for use in the practice of this invention, whether or not the package has actually been subjected to the API GL-4 performance tests.

Typically, the lubricant of the invention further comprises a gear oil additive package comprising at least one oil-soluble basic nitrogen-containing ashless dispersant and an oil-soluble phosphorus and sulphur-containing antiwear and/or extreme pressure additive complement comprising (1) at least one oil-soluble metal-free sulphur-containing antiwear and/or extreme pressure agent in which the sulphur is bonded to carbon or to more sulphur and (2) at least one oil-soluble metal-free phosphorus-containing antiwear and/or extreme pressure agent, wherein the dispersant and the metal-free sulphur-containing antiwear and/or extreme pressure agent are proportioned such that the mass ratio (wt/wt) of nitrogen in the dispersant to sulphur in the sulphur-containing antiwear and/or extreme pressure agent is in the range of 0.0005:1 to 0.5:1, and the dispersant and the metal-free phosphorus-containing antiwear and/or extreme pressure agent are proportioned such that the mass ratio (wt/wt) of nitrogen in the dispersant to phosphorus in the metal-free phosphorus-containing antiwear and/or extreme pressure agent is in the range of 0.005:1 to 5:1.

In a further embodiment, the present invention comprises use of at least one overbased alkaline earth metal sulphurised phenate or salicylate to improve the frictional properties of a lubricant suitable for use as a gear oil lubricant for a manual transmission of the synchroniser type, which comprises a base oil as defined above, the lubricant being essentially free of any metal additive component other than the phenate or salicylate and having on a weight basis a boron content of not more than 1,000 ppm.

In a further embodiment, the present invention provides a gear oil additive concentrate which comprises (1) an oil-soluble phosphorus and sulphur-containing antiwear and/or extreme pressure additive complement and (2) at least one overbased alkaline earth metal sulphurised phenate or salicylate wherein, when blended with a base oil as defined above to form a lubricant containing from 0.01 to 2 wt% of said phenate or salicylate, the gear oil additive concentrate provides a lubricant which has a kinematic viscosity at 100°C in the range of 4 to 32mm².s⁻¹ (cSt), which is suitable for use as a gear oil lubricant for a manual transmission of the synchroniser type, which contains up to 100 ppm of metal additive component other than the phenate or salicylate, and which has a boron content of not more than 1,000 ppm.

Typically, when blended with the said base oil, the said gear oil additive concentrate provides a lubricant which contains no metal additive other than the phenate or salicylate, and which has a boron content of not more than 300 ppm.

Typically, the gear oil additive concentrate further comprises at least one oil-soluble basic nitrogen-containing ashless dispersant, preferably a succinimide ashless dispersant and/or a succinic ester-amide ashless dispersant, and more preferably a Mannich base ashless dispersant. The oil-soluble phosphorus and sulfur-containing antiwear and/or extreme pressure additive complement of such compositions is preferably composed of (1) at least one oil-soluble metal-free sulphur-containing antiwear and/or extreme pressure agent in which the sulfur is bonded to carbon or to more sulfur, and (2) at least one oil-soluble metal-free phosphorus-containing antiwear and/or extreme pressure agent. In these embodiments, the dispersant and the metal-free sulphur-containing antiwear and/or extreme pressure agent are proportioned such that the mass ratio (wt/wt) of nitrogen in the dispersant to sulphur in the sulphur-containing antiwear and/or extreme pressure agent is in the range of about 0.0005:1 to about 0.5:1, and preferably in the range of about 0.003:1 to about 0.2:1. Likewise the dispersant and the metal-free phosphorus-containing antiwear and/or extreme pressure agent are proportioned such that the mass ratio (wt/wt) of nitrogen in the dispersant to phosphorus in the metal-free phosphorus-containing antiwear and/or extreme pressure agent is in the range of about 0.005:1 to about 5:1, and preferably in the range of about 0.01:1 to about 2:1. In each of these embodiments the gear oil additive package (concentrate) or gear lubricant preferably has a boron content such that the finished lubricant contains by weight up to 1,000 ppm, preferably up to 300 ppm, and most preferably not more than 25 ppm of boron. One preferred way of introducing at least a portion of such boron is to provide additive packages and finished lubricants compositions containing a borated basic nitrogen-containing ashless dispersant.

In additional embodiments, any of the above additive concentrates and finished lubricant compositions further comprise at least one oil-soluble demulsifying agent.

Preferably the lubricant compositions of this invention have a halogen content, if any, of no more than 100 ppm, and more preferably no more than 50 ppm on a weight basis.

In each of the embodiments of this invention, the overbased metal phenate or salicylate can be employed as a separate component (e.g., as a "top-treat" to the base oil with which the additive package has been or will be blended) or as a component of the additive package itself. Similarly, while use of additive packages is preferred, it is possible to blend the overbased metal sulfurized phenate and/or salicylate and the respective components of the additive package into the base oil individually or in various compatible sub-combinations.

### Base Oils.

Most poly-alpha-olefin oils are formed by oligomerization or co-oligomerization of 1-alkene hydrocarbon having 6 to 20 and preferably 8 to 16 carbon atoms in the molecule and hydrogenation of the resultant oligomer. In some cases, a suitable poly-alpha-olefin oils can be co-oligomers of a short chain 1-olefin such as ethylene and one or more longer chain alpha-olefins, such as for example the product available from Mitsui Petrochemical Company, Ltd. under the LUCANT trademark. Hydrogenated poly-alpha-olefin oils formed from 1-decene are particularly preferred. Methods for the production of liquid 1-alkene hydrocarbon oils are known and reported in the literature. See for example U. S. Pat. Nos. 3,763,244; 3,780,128; 4,172,855; 4,218,330; and 4,950,822.

Synthetic ester oils are available in the marketplace. Typical synthetic ester oils include such materials as the esters of dicarboxylic acids (e.g., phthalic acid, succinic acid, maleic acid, azelaic acid, suberic acid, sebacic acid, fumaric acid, adipic acid, linoleic acid dimer) with a variety of alcohols (e.g., butyl alcohol, hexyl alcohol, dodecyl alcohol, 2-ethylhexyl alcohol, ethylene glycol). Specific examples of these esters include dibutyl adipate, di(1-ethylpropyl) adipate, di(1,3-dimethylbutyl) adipate, di(2-ethylhexyl) adipate, didodecyl adipate, di(tridecyl) adipate, di(2-ethylhexyl) sebacate, dilauryl sebacate, di-n-hexyl fumarate, dioctyl sebacate, di(1-methylpropyl) azelate, diisooctyl azelate, diisodecyl azelate, dioctyl phthalate, didecyl phthalate, mixed C₉ and C₁₁ dialkyl phthalate, dibutyl sebacate, di(1-ethylpropyl) sebacate, di(eicosyl) sebacate, the 2-ethylhexyl diester of linoleic acid dimer, and the complex ester formed by reacting one mole of sebacic acid with two moles of tetraethylene glycol and two moles of 2-ethylhexanoic acid. Other synthetic esters which may be used as synthetic oils include those made from C₃-C₁₂ monocarboxylic acids and polyols and polyol ethers such as neopentyl glycol, trimethylolpropane, pentaerythritol and dipentaerythritol. Trimethylol propane tripelargonate and pentaerythritol tetracaproate serve as examples.

The base oils may contain as optional blending components a mineral oil or other suitable oleaginous liquid of lubricating viscosity, provided the overall base lubricant satisfies the proportions and viscosity parameters given above, and is suitable for use in forming a finished gear lubricant that satisfies or exceeds the specifications for API GL-4 service, and provided further that the resultant finished oil remains amenable to friction improvement pursuant to this invention. Suitable mineral oils include those of appropriate viscosity refined from crude oil of any source including Gulf Coast, Midcontinent, Pennsylvania, California, Alaska, Middle East, North Sea and the like. Standard refinery operations may be used in processing the mineral oil. Among the general types of petroleum oils useful in the compositions of this invention are solvent neutrals, bright stocks, cylinder stocks, residual oils, hydrocracked base stocks, hydrotreated oils, partially hydrotreated oils, paraffin oils including pale oils, and solvent extracted naphthenic oils. Such oils and blends of them are produced by a number of conventional techniques known to those skilled in the art. Suitable reprocessed or reclaimed mineral oil base stocks may also be used. Most gear oil packages contain diluent oils or solvents for certain active ingredients or components. However, since such diluent oils or solvents are added to the base oil along with the additive package or with one or more additive components blended separately or individually into the base oil, such diluent oils or solvents are to be omitted from consideration when assessing the makeup of the base oil of the compositions of this invention.

### Overbased Phenate or Salicylate

Overbased alkaline earth metal sulfurized phenates are also known as overbased alkaline earth metal phenol sulfides. These materials as well as overbased alkaline earth metal salicylates are available as articles of commerce. Of the overbased alkaline earth phenates and salicylates, the magnesium compounds are a preferred group. The most preferred however are the overbased calcium phenates and salicylates. As between overbased phenates and overbased salicylates, the phenates are preferred. As is known, these overbased materials contain more than a stoichiometric amount of the metal. Methods for producing such materials have been reported in the patent literature. Test work has shown that the additive must be overbased, and for good performance the phenate should have a total base number (TBN) of at least 200 and preferably at least about 250. The salicylate should have a TBN of at least 150. TBN is measured using the ASTM D2896 procedure, and represents mg of KOH per gram of sample.

Quantities ranging from as little as 0.01 wt% up to as much as 2 wt% of the overbased metal phenate or salicylate (or combination thereof) based on the total weight of the finished lubricant can be employed. Ordinarily the amount used will not be greatly in excess of that amount needed to yield the friction performance desired in the particular finished gear oil lubricant in question. In most cases the amount will not be above 1 wt%, and often will not exceed 0.5 wt%. In the case of the friction-improved additive packages of this invention, the amount will be proportioned such that when the package is blended into the base oil at the recommended or desired concentration, the resultant finished oil will contain the above-specified amount of the overbased phenate or salicylate. These proportions of the overbased metal phenate or salicylate are based on the active ingredient, and thus the weight of any solvent or diluent associated with the overbased phenate or salicylate as used should be subtracted from the additive weight when calculating the concentration of the overbased metal phenate or salicylate in the finished oil or in the friction-improved additive package. However the total weight of the finished oil or of the completed additive package will include the weight of such solvent or diluent.

### Additive Packages

The specifications for API GL-4 and API GL-5 service are published in ASTM Publication STP-512A entitled "Laboratory Performance Tests for Automotive Gear Lubricants" (March 1987).

A number of gear oil additive packages (concentrates) that provide API GL-4 or API GL-5 performance are available in the marketplace. They generally contain at least a sulfur-phosphorus antiwear or extreme pressure additive system, one or more antioxidants, one or more corrosion inhibitors, and an antifoam additive and may, preferably do, contain a dispersant additive.

### ZF Synchronizer Test

As is known in the art, the ZF Synchronizer test has been designed for the evaluation of oil performance in commercially available synchromesh units under endurance conditions with the bulk lubricant temperature controlled at a relatively high level. While it is important to simulate fairly closely the actual conditions met in service, the need to produce a test result in an acceptable period has to be taken into account. Briefly, two halves of a transmission synchromesh unit are repeatedly brought together under conditions of known force and speed differential until failure occurs. Failure may be defined in terms of synchromesh performance or overall wear. The test rig used in the procedure was designed with consideration of work done by Socin and Walters, SAE Paper Number 680008 entitled "Manual Transmission Synchronizers"; Fano, CEC TLPG4 Chairman's Final Report, 1985, entitled "Synchromesh Test Method With Proposed Synchro Test Rig"; and Brugen, Thies and Naurian of Zahnradfabrik Friedrichshafen A.G. in a paper entitled "Einfluss Des Schmierstoffes auf die Schaltelemente Von Fahrzeuggetrieben". The two synchromesh units are assembled in a gear box which forms the oil reservoir and facilitates splash lubrication of components. Drive may be transmitted along the main shaft or via the layshaft gears to give an increased ratio. The input speed is kept constant by means of a DC drive control system and a large flywheel simulating vehicle inertia. On changing gear, the output shaft accelerates and decelerates the small flywheel which simulates clutch inertia. A pivot linkage connected to a pneumatic cylinder provides the actuating force which is measured by means of a load ring strain gauge. A small heater is used to control oil temperature.

Torque transmitted through the output shaft can be measured to give an indication of the coefficient of friction between the synchronizing cones. The synchromesh units used are standard commercially available steel units with a molybdenum-based plasma spray coating on the inner surface of the outer synchro-ring. The synchromesh units are renewed before each test. Typically, when measured at a point of relatively high torque during a gear change, the coefficient of friction for satisfactory synchronizer performance in the test is at least 0.065.

Another performance criterion which may be used when performing the test for qualification purposes is excessive vibration of the gear box casing in the axial plane, a condition symptomatic of poor gear changes. For this purpose the control and monitoring of the rig is coordinated by a process controller. During a test the number of poor changes is recorded. The test is terminated prematurely if this number becomes unacceptable or the vibration becomes excessively harsh.

Test components may be evaluated by inspecting the friction surface of the inner synchronizer cone using a Perthometer stylus device both before and after test. Polishing of the metal surface or the build up of a glaze of decomposed lubricant or additive yields an unacceptably smooth surface finish. This in turn causes low frictional values during the gear change and can lead to clash of the sleeve and gear clutch teeth. Wear measurements are also made on the test components.

### Performance

The following examples illustrate, inter alia, the dramatic improvements in performance that are made possible by the practice of this invention. These examples are not intended to limit, and should not be construed as limiting, this invention. In the examples, all percentages are by weight.

### Example

ZF Synchronizer tests were performed under the same conditions using a lubricant of this invention and a control lubricant made from the same components with but one exception: the composition of this invention contained 0.5% (approximately 0.3% on an active ingredient basis) of an overbased calcium sulfurized alkyl phenate having a nominal TBN of 250 ("Phenate"), whereas the control contained no such component. The base oils were fully synthetic oil blends of two PAO fluids having nominal viscosities at 100°C of 8 and 40 cSt (mm².s⁻¹), and a synthetic ester, namely bis(tridecyl)adipate ("DTDA"). Each lubricant contained the same quantity of the same metal-free and boron-free API GL-4 additive package (HiTEC 381, available from Ethyl Corporation). The proportions of these components are summarised in the following table:

| Components | Control Composition, % | Invention Composition, % |
|---|---|---|
| PAO, 8 mm².s⁻¹ | 70.25 | 69.75 |
| PAO, 40 mm².s⁻¹ | 16.00 | 16.00 |
| DTDA | 10.00 | 10.00 |
| API GL-4 Package | 3.75 | 3.75 |
| Phenate | None | 0.50 |

The control composition had a kinematic viscosity at 100°C of 9.53mm².s⁻¹. The composition of the invention had a kinematic viscosity at 100°C of 9.55mm².s⁻¹.

The control composition was able to complete only 792 cycles in the test. The test had to be shut down at that point because very harsh bad gear changes had occurred and the coefficient of friction had already fallen to below 0.05. In sharp contrast, the composition of this invention successfully completed 50,000 cycles, and during the entire test the coefficient of friction remained consistently above 0.065.

## Claims

1. A lubricant suitable for use as a gear oil lubricant for a manual transmission of the synchroniser type having a kinematic viscosity at 100°C in the range of 4 to 32 mm².s⁻¹ (cSt), and comprising:
a) a base oil comprising more than 40% by volume of hydrogenated poly-α-olefin oil; and
b) a friction improving amount in the range of 0.01 to 2wt% based on the total weight of the lubricant of at least one overbased alkaline earth metal sulphurised phenate or salicylate;
the lubricant being essentially free of any metal additive component other than the phenate or salicylate, and having on a weight basis a boron content of not more than 1,000 ppm.

2. A lubricant according to claim 1 which does not contain any metal-containing additive component other than the phenate or salicylate, and which has on a weight basis a boron content of not more than 300 ppm.

3. A lubricant according to claim 1 or 2 which has a boron content of not more than 25 ppm.

4. A lubricant according to any one of claims 1 to 3 which does not contain boron.

5. A lubricant according to any one of claims 1 to 4 wherein component b) is at least one overbased alkaline earth metal sulphurised phenate having a TBN of at least 200.

6. A lubricant according to claim 5 wherein the phenate is an overbased calcium sulphurised phenate having a nominal TBN of 250.

7. A lubricant according to any one of claims 1 to 6 wherein the base oil
a) comprises (i) at least 40% by weight of hydrogenated poly-α-olefin oil; (ii) 5 to 25% by weight of synthetic ester oil, and (iii) 0 to 55% by weight of mineral oil.

8. A lubricant according to any one of claims 1 to 7 which further comprises a gear oil additive package comprising at least one oil-soluble basic nitrogen-containing ashless dispersant and an oil-soluble phosphorus and sulphur-containing antiwear and/or extreme pressure additive complement comprising (1) at least one oil-soluble metal-free sulphur-containing antiwear and/or extreme pressure agent in which the sulphur is bonded to carbon or to more sulphur and (2) at least one oil-soluble metal-free phosphorus-containing antiwear and/or extreme pressure agent, wherein the dispersant and the metal-free sulphur-containing antiwear and/or extreme pressure agent are proportioned such that the mass ratio (wt/wt) of nitrogen in the dispersant to sulphur in the sulphur-containing antiwear and/or extreme pressure agent is in the range of 0.0005:1 to 0.5:1, and the dispersant and the metal-free phosphorus-containing antiwear and/or extreme pressure agent are proportioned such that the mass ratio (wt/wt) of nitrogen in the dispersant to phosphorus in the metal-free phosphorus-containing antiwear and/or extreme pressure agent is in the range of 0.005:1 to 5:1.

9. A lubricant according to any one of claims 1 to 8 having on a weight basis a halogen content of no more than 100ppm.

10. Use, in a manual transmission of the synchronizer type, of a lubricant according to any one of claims 1 to 9 to improve transmission performance during operation under service conditions.

11. Use of at least one overbased alkaline earth metal sulphurised phenate or salicylate to improve the frictional properties of a lubricant suitable for use as a gear oil lubricant for a manual transmission of the synchroniser type, which comprises a base oil as defined in claim 1 or 7, the lubricant being essentially free of any metal additive component other than the phenate or salicylate and having on a weight basis a boron content of not more than 1,000 ppm.

12. Use according to claim 11, wherein the lubricant comprises from 0.01 to 2 wt% based on the total weight of the lubricant of overbased sulphurised phenate or salicylate.

13. A gear oil additive concentrate which comprises (1) an oil-soluble phosphorus and sulphur-containing antiwear and/or extreme pressure additive complement and (2) at least one overbased alkaline earth metal sulphurised phenate or salicylate wherein, when blended with a base oil as defined in claim 1 or 7 to form a lubricant containing from 0.01 to 2 wt% of said phenate or salicylate, the gear oil additive concentrate provides a lubricant which has a kinematic viscosity at 100°C in the range of 4 to 32mm².s⁻¹ (cSt), which is suitable for use as a gear oil lubricant for a manual transmission of the synchroniser type, which contains up to 100 ppm of metal additive component other than the phenate or salicylate, and which has a boron content of not more than 1,000 ppm.

14. A gear oil additive concentrate according to claim 13 which when blended with base oil provides a lubricant which contains no metal additive other than the phenate or salicylate, and which has a boron content of not more than 300 ppm.

15. A gear oil additive concentrate according to claim 13 or 14 additionally comprising at least one oil-soluble basic nitrogen-containing ashless dispersant and in which the oil-soluble phosphorus and sulphur-containing antiwear and/or extreme pressure additive complement of the concentrate comprises (1) at least one oil-soluble metal-free sulphur-containing antiwear and/or extreme pressure agent in which the sulphur is bonded to carbon or to more sulphur, and (2) at least one oil-soluble metal-free phosphorus-containing antiwear and/or extreme pressure agent wherein the dispersant and the metal-free sulphur-containing antiwear and/or extreme pressure agent are proportioned such that the mass ratio (wt/wt) of nitrogen in the dispersant to sulphur in the sulphur-containing antiwear and/or extreme pressure agent is in the range of 0.0005:1 to 0.5:1, and the dispersant and the metal-free phosphorus-containing antiwear and/or extreme pressure agent are proportioned such that the mass ratio (wt/wt) of nitrogen in the dispersant to phosphorus in the metal-free phosphorus-containing antiwear and/or extreme pressure agent is in the range of 0.005:1 to 5:1.

## Patentansprüche

1. Schmiermittel, das sich zur Verwendung als Getriebeölschmiermittel für Schaltgetriebe vom Synchrontyp eignet, eine kinematische Viskosität bei 100°C im Bereich von 4 bis 32 mm² · s⁻¹ (cSt) hat und umfasst:
a) ein Grundöl, das mehr als 40 Vol.-% hydriertes Poly-α-olefinöl umfasst und
b) eine die Reibung verbessernde Menge im Bereich von 0,01 bis 2 Gew.-%, bezogen auf das Gesamtgewicht des Schmiermittels, mindestens eines überbasischen geschwefelten Erdalkalimetallphenats oder -salicylats,
wobei das Schmiermittel im Wesentlichen frei von irgendwelchen Metalladditivkomponenten außer dem Phenat oder Salicylat ist und auf Gewichtsbasis einen Borgehalt von nicht mehr als 1.000 ppm hat.

2. Schmiermittel nach Anspruch 1, das außer dem Phenat oder Salicylat keinerlei metallhaltige Additivkomponente enthält und auf Gewichtsbasis einen Borgehalt von nicht mehr als 300 ppm hat.

3. Schmiermittel nach Anspruch 1 oder 2, das einen Borgehalt von nicht mehr als 25 ppm hat.

4. Schmiermittel nach einem der Ansprüche 1 bis 3, das kein Bor enthält.

5. Schmiermittel nach einem der Ansprüche 1 bis 4, in dem die Komponente b) mindestens ein überbasisches geschwefeltes Erdalkalimetallphenat mit einer TBN (Gesamtbasenzahl) von mindestens 200 ist.

6. Schmiermittel nach Anspruch 5, in dem das Phenat ein überbasisches geschwefeltes Calciumphenat mit einer nominellen TBN von 250 ist.

7. Schmiermittel nach einem der Ansprüche 1 bis 6, in dem das Grundöl a) (i) mindestens 40 Gew.-% eines hydrierten Poly-α-olefinöls; (ii) 5 bis 25 Gew.-% Öl aus einem synthetischen Ester und (iii) 0 bis 55 Gew.-% Mineralöl enthält.

8. Schmiermittel nach einem der Ansprüche 1 bis 7, das außerdem ein Getriebeöladditivpaket umfasst, das mindestens ein öllösliches basisches stickstoffhaltiges aschefreies Dispergiermittel und ein öllösliches phosphor- und schwefelhaltiges Antiverschleiß- und/oder Hochdruck-Additivergänzungsmittel umfasst, umfassend (1) mindestens ein öllösliches metallfreies schwefelhaltiges Antiverschleiß- und/oder Hochdruckmittel, in dem der Schwefel an Kohlenstoff oder weiteren Schwefel gebunden ist, und (2) mindestens ein öllösliches metallfreies phosphorhaltiges Antiverschleiß- und/ oder Hochdruckmittel, in dem das Dispergiermittel und das metallfreie schwefelhaltige Antiverschleiß- und/oder Hochdruckmittel in einem solchen Verhältnis gewählt werden, dass das Massenverhältnis (Gewicht/Gewicht) von Stickstoff im Dispergiermittel zu Schwefel im schwefelhaltigen Antiverschleiß- und/oder Hochdruckmittel im Bereich von 0,0005 : 1 bis 0,5 : 1 liegt und das Verhältnis des Dispergiermittels und des metallfreien phosphorhaltigen Antiverschleiß- und/oder Hochdruckmittels so gewählt wird, dass das Massenverhältnis (Gewicht/Gewicht) von Stickstoff im Dispergiermittel zu Phosphor im metallfreien phosphorhaltigen Antiverschleiß- und/oder Hochdruckmittel im Bereich von 0,005 : 1 bis 5 : 1 liegt.

9. Schmiermittel nach einem der Ansprüche 1 bis 8, das auf Gewichtsbasis einen Halogengehalt von nicht mehr als 100 ppm hat.

10. Verwendung eines Schmiermittels nach einem der Ansprüche 1 bis 9 in einem Schaltgetriebe vom Synchrontyp, um die Getriebeleistung während des Betriebs unter Betriebsbedingungen zu verbessern.

11. Verwendung mindestens eines überbasischen geschwefelten Erdalkalimetallphenats oder -salicylats zur Verbesserung der Reibungseigenschaften eines Schmiermittels, das zur Verwendung als Getriebeschmieröl für ein Schaltgetriebe vom Synchrontyp geeignet ist und ein in Anspruch 1 oder 7 definiertes Grundöl umfasst, wobei das Schmiermittel außer dem Phenat oder Salicylat im Wesentlichen frei von allen Metalladditivkomponenten ist und auf Gewichtsbasis einen Borgehalt von nicht mehr als 1.000 ppm hat.

12. Verwendung nach Anspruch 11, in der das Schmiermittel bezogen auf das Gesamtgewicht des Schmiermittels 0,01 bis 2 Gew.-% überbasisches geschwefeltes Phenat oder Salicylat enthält.

13. Getriebeöladditivkonzentrat, umfassend: (1) ein öllösliches phosphor- und schwefelhaltiges Antiverschleiß- und/oder Hochdruck-Additivergänzungsmittel und (2) mindestens ein überbasisches geschwefeltes Erdalkalimetallphenat oder -salicylat, in dem das Getriebeöladditivkonzentrat dann, wenn es mit einem Grundöl wie in Anspruch 1 oder 7 definiert gemischt wird, um ein Schmiermittel zu bilden, das 0,01 bis 2 Gew.-% des Phenats oder Salicylats enthält, ein Schmiermittel mit einer kinematischen Viskosität bei 100°C im Bereich von 4 bis 32 mm²·s⁻¹ (cSt) zur Verfügung stellt, das zur Verwendung als Getriebeölschmiermittel für ein Schaltgetriebe vom Synchrontyp geeignet ist, bis zu 100 ppm einer anderen Metalladditivkomponente außer Phenat oder Salicylat enthält und einen Borgehalt von nicht mehr als 1.000 ppm hat.

14. Getriebeöladditivkonzentrat nach Anspruch 13, das dann, wenn es mit einem Grundöl gemischt wird, ein Schmiermittel zur Verfügung stellt, das außer dem Phenat oder Salicylat kein Metalladditiv enthält und einen Borgehalt von nicht mehr als 300 ppm hat.

15. Getriebeöladditivkonzentrat nach Anspruch 13 oder 14, das außerdem mindestens ein öllösliches basisches stickstoffhaltiges aschefreies Dispergiermittel umfasst und in dem das öllösliche phosphor- und schwefelhaltige Antiverschleiß- und/oder Hochdruck-Additivergänzungsmittel des Konzentrats umfasst: (1) mindestens ein öllösliches metallfreies schwefelhaltiges Antiverschleiß- und/oder Hochdruckmittel, in dem der Schwefel an Kohlenstoff oder weiteren Schwefel gebunden ist, und (2) mindestens ein öllösliches metallfreies phosphorhaltiges Antiverschleiß- und/oder Hochdruckmittel, in dem das Dispergiermittel und das metallfreie schwefelhaltige Antiverschleiß- und/oder Hochdruckmittel in einem solchen Verhältnis gewählt werden, dass das Massenverhältnis (Gewicht/Gewicht) von Stickstoff im Dispergiermittel zu Schwefel im schwefelhaltigen Antiverschleiß- und/ oder Hochdruckmittel im Bereich von 0,0005 : 1 bis 0,5 : 1 liegt und das Dispergiermittel und das metallfreie phosphorhaltige Antiverschleiß- und/oder Hochdruckmittel in einem solchen Verhältnis gewählt werden, dass das Massenverhältnis (Gewicht/ Gewicht) von Stickstoff im Dispergiermittel zu Phosphor im metallfreien phosphorhaltigen Antiverschleiß- und/oder Hochdruckmittel im Bereich von 0,005 : 1 bis 5 : 1 liegt.

## Revendications

1. Lubrifiant apte à être utilisé comme huile lubrifiante d'engrenages pour une transmission manuelle du type synchroniseur, ayant une viscosité cinématique à 100°C comprise dans l'intervalle de 4 à 32 mm².s⁻¹ (cSt), et comprenant :
a) une huile de base comprenant plus de 40 % en volume d'une huile poly-α-oléfinique hydrogénée ; et
b) une quantité modificatrice de frottement comprise dans l'intervalle de 0,01 à 2 % en poids, sur la base du poids total du lubrifiant, d'au moins un phénate ou salicylate sulfuré de métal alcalino-terreux surbasique ;
le lubrifiant étant pratiquement dépourvu de tout constituant additif métallique autre que le phénate ou salicylate, et ayant, sur base pondérale, une teneur en bore non supérieure à 1000 ppm.

2. Lubrifiant suivant la revendication 1, qui ne contient aucun constituant additif contenant un métal, autre que le phénate ou salicylate, et qui a, sur base pondérale, une teneur en bore non supérieure à 300 ppm.

3. Lubrifiant suivant la revendication 1 ou 2, qui a une teneur en bore non supérieure à 25 ppm.

4. Lubrifiant suivant l'une quelconque des revendications 1 à 3, qui ne contient pas de bore.

5. Lubrifiant suivant l'une quelconque des revendications 1 à 4, dans lequel le constituant b) consiste en au moins un phénate sulfuré de métal alcalino-terreux surbasique ayant un IBT d'au moins 200.

6. Lubrifiant suivant la revendication 5, dans lequel le phénate est un phénate sulfuré de calcium surbasique ayant un IBT nominal de 250.

7. Lubrifiant suivant l'une quelconque des revendications 1 à 6, dans lequel l'huile de base a) comprend (i) au moins 40 % en poids d'une huile poly-α-oléfinique hydrogénée ; (ii) 5 à 25 % en poids d'une huile du type ester synthétique, et (iii) 0 à 55 % en poids d'une huile minérale.

8. Lubrifiant suivant l'une quelconque des revendications 1 à 7, qui comprend en outre une formulation d'additifs pour huile d'engrenages, comprenant au moins un dispersant sans cendres azoté basique soluble dans l'huile et un complément additif anti-usure et/ou extrême-pression contenant du phosphore et du soufre, soluble dans l'huile, comprenant (1) au moins un agent anti-usure et/ou extrême-pression contenant du soufre et dépourvu de métaux, soluble dans l'huile, dans lequel le soufre est lié au carbone ou à une quantité supplémentaire de soufre, et (2) au moins un agent anti-usure et/ou extrême-pression contenant du phosphore et dépourvu de métaux, soluble dans l'huile, dans lequel le dispersant et l'agent anti-usure et/ou extrême-pression contenant du soufre et dépourvu de métaux sont présents en des proportions telles que le rapport en masse (poids/poids) de l'azote dans le dispersant au soufre dans l'agent anti-usure et/ou extrême-pression contenant du soufre soit compris dans l'intervalle de 0,0005:1 à 0,5:1, et le dispersant et l'agent anti-usure et/ou extrême-pression contenant du phosphore et dépourvu de métaux sont présents en des proportions telles que le rapport en masse (poids/poids) de l'azote dans le dispersant, au phosphore dans l'agent anti-usure et/ou extrême-pression contenant du phosphore et dépourvu de métaux, soit compris dans l'intervalle de 0,005:1 à 5:1.

9. Lubrifiant suivant l'une quelconque des revendications 1 à 8, ayant sur base pondérale, une teneur en halogène non supérieure à 100 ppm.

10. Utilisation, dans une transmission manuelle du type synchroniseur, d'un lubrifiant suivant l'une quelconque des revendications 1 à 9 pour améliorer les performances de transmission au cours du fonctionnement dans les conditions d'utilisation.

11. Utilisation d'au moins un phénate ou salicylate sulfuré de métal alcalino-terreux surbasique pour améliorer les propriétés de frottement d'un lubrifiant apte à l'utilisation comme huile lubrifiante d'engrenages pour une transmission manuelle du type synchroniseur, qui comprend une huile de base répondant à la définition suivant la revendication 1 ou 7, le lubrifiant étant pratiquement dépourvu de tout constituant additif métallique autre que le phénate ou salicylate et ayant, sur base pondérale, une teneur en bore non supérieure à 1000 ppm.

12. Utilisation suivant la revendication 11, dans laquelle le lubrifiant comprend 0,01 à 2 % en poids, sur la base du poids total du lubrifiant, d'un phénate ou salicylate sulfuré surbasique.

13. Concentré d'additifs pour huile d'engrenages, qui comprend (1) un complément additif anti-usure et/ou extrême-pression contenant du phosphore et du soufre, soluble dans l'huile, et (2) au moins un phénate ou salicylate sulfuré de métal alcalino-terreux surbasique, dans lequel, lorsqu'il est mélangé à une huile de base répondant à la définition suivant la revendication 1 ou 7 pour former un lubrifiant contenant 0,01 à 2 % en poids dudit phénate ou salicylate, le concentré d'additifs pour huile d'engrenages donne un lubrifiant ayant une viscosité cinématique à 100°C comprise dans l'intervalle de 4 à 32 mm².s⁻¹ (cSt), qui est apte à l'utilisation comme huile lubrifiante d'engrenages pour une transmission manuelle du type synchroniseur, qui contient jusqu'à 100 ppm de constituant additif métallique autre que le phénate ou salicylate, et qui a une teneur en bore non supérieure à 1000 ppm.

14. Concentré d'additifs pour huile d'engrenages suivant la revendication 13, qui, lorsqu'il est mélangé à une huile de base, donne un lubrifiant qui ne contient aucun additif métallique autre que le phénate ou salicylate, et qui a une teneur en bore non supérieure à 300 ppm.

15. Concentré d'additifs pour huile d'engrenages suivant la revendication 13 ou 14, comprenant en outre au moins un dispersant sans cendres azoté basique soluble dans l'huile, et dans lequel le complément additif anti-usure et/ou extrême-pression contenant du phosphore et du soufre, soluble dans l'huile, du concentré comprend (1) au moins un agent anti-usure et/ou extrême-pression contenant du soufre, dépourvu de métaux, soluble dans l'huile, dans lequel le soufre est lié au carbone ou à une quantité supplémentaire de soufre, et (2) au moins un agent anti-usure et/ou extrême-pression contenant du phosphore et dépourvu de métaux, soluble dans l'huile, dans lequel le dispersant et l'agent anti-usure et/ou extrême-pression contenant du soufre et dépourvu de métaux sont présents en des proportions telles que le rapport en masse (poids/poids) de l'azote dans le dispersant au soufre dans l'agent anti-usure et/ou extrême-pression contenant du soufre soit compris dans l'intervalle de 0,0005:1 à 0,5:1, et le dispersant et l'agent anti-usure et/ou extrême-pression contenant du phosphore et dépourvu de métaux sont présents en des proportions telles que le rapport en masse (poids/poids) de l'azote dans le dispersant, au phosphore dans l'agent anti-usure et/ou extrême-pression contenant du phosphore et dépourvu de métaux, soit compris dans l'intervalle de 0,005:1 à 5:1.
